

## UNITED STATES PATENT OFFICE

2,388,816

## PHOTOGRAPHIC DEVELOPER

Frederic R. Bean, Rochester, N. Y., assignor to  
 Eastman Kodak Company, Rochester, N. Y., a  
 corporation of New Jersey

No Drawing. Application June 25, 1942,  
 Serial No. 448,415

15 Claims. (Cl. 95—88)

This invention relates to photographic developing solutions and more particularly to concentrated photographic developing solutions and dry mixtures of chemicals suitable for dissolving in water to form photographic developing solutions.

In making concentrated solutions of photographic developing compounds, reagents such as polyhydric alcohols, amino alcohols, and caustic alkalis have been used singly or in combinations to act as solubilizing agents for the developer in the presence of sodium sulfite. When caustic alkali is used the developing solutions tend to have poor keeping properties, when amino alcohols are used the solutions may give fog and the polyhydric alcohols are not especially good solvents for sodium sulfite.

I have found a class of compounds useful in making developer solutions, especially compositions in the solid or concentrated form, which compounds have not only a solubilizing action on the ingredients of the developer but also act as preservatives and prevent formation of sludge during development.

Compounds useful in developing solutions according to my invention are the alkali metal salts of aminomethane sulfonates and of aminomethane sulfonates as, for example, the sodium salts of  $\beta$ -hydroxyethylaminomethane sulfonates, di-( $\beta$ -hydroxyethyl) aminomethane sulfonate, ethylenediamino-bis-methane sulfonate,  $\beta$ -hydroxyethylaminodimethylmethane sulfonate, cyclohexylaminomethane sulfonate, morpholinomethane sulfonate, p-carboxyphenylaminomethane sulfonate and sulfinate, ethylenediamino-bis-methane sulfonate, ethylenediamino-bis-dimethylmethane sulfonate, carboxymethylaminomethane sulfonate, etc. In addition mixtures of aminomethane sulfonates and sulfonates are suitable for use in developer compositions.

The aminomethane sulfonate compounds of my invention may be prepared from aldehydes or ketones by reaction with sodium bisulfite and an amino compound, or by reaction of formaldehyde or other aldehyde or ketone bisulfite compound with an amine.

The structure of a typical aminomethane sulfonate, that is sodium- $\beta$ -hydroxyethylaminomethane sulfonate, is believed to be the following:



A suitable method of preparation of the above compound is as follows: 75 cc. of 40% formaldehyde are added to 150–200 cc. of water and then 104 grams of sodium bisulfite are then added. To this solution are added 61 grams of monoethanol-

amine and the solution is warmed at about 50°–60° C. for about 30 minutes. If desired, one mole of solid sodium formaldehyde-bisulfite may be caused to react with the monoethanolamine in a similar manner. The resulting product may be isolated and added to a photographic developing solution, or if desired, the photographic ingredients may be added to the above solution and made up to the required volume by the addition of water.

In a similar manner di-( $\beta$ -hydroxyethyl) aminomethane sulfonate may be prepared as follows: 420 grams of diethanolamine and 536 grams of sodium formaldehyde bisulfite are placed in 300–400 cc. of water and the mixture is warmed at about 50°–60° C. for 30 minutes and allowed to stand overnight at room temperature. The reaction product may be isolated from the resulting syrupy reaction mixture by the addition of organic solvents such as acetone, methyl alcohol, tertiary butyl alcohol, etc., which cause the reaction product to precipitate out as fine white crystals.

Aminomethane sulfonates of ketones capable of reacting with sodium bisulfite may be prepared in a manner analogous to those above-described by the reaction of an amine with a ketone and sodium bisulfite or a ketone-bisulfite compound, by heating for a suitable length of time.

The aminomethane sulfonate compounds of the invention may, for instance, be prepared by reaction of an amino compound with aldehyde sulfonates such as formaldehyde sulfoxalate. A typical aminomethane sulfonate compound useful in my invention, that is, di-sodium-p-carboxyphenylaminomethane sulfonate, may be prepared as follows: 34.2 grams of p-aminobenzoic acid are added to 30–40 cc. of water containing 10 grams of sodium hydroxide. Thereafter, 38.5 grams of formaldehyde sulfoxalate are added to the hot solution and the mixture heated at 60°–70° C. for 1–2 hours. After cooling the reaction product is precipitated from the syrupy mixture by the addition of acetone.

Other aminomethane sulfonates are prepared in a similar manner by reaction of other amino compounds with formaldehyde sulfoxalate, or other sulfoxalates as, for example, prepared by the reduction of aminomethane sulfonates.

A method of preparing a mixture of aminomethane sulfonate and an aminomethane sulfonate compound is given as follows: molecular proportions of formaldehyde and sodium hydrosulfite are caused to react in aqueous solution, and thereafter, the product consisting of sodium formaldehyde sulfoxalate and sodium formaldehyde bisulfite is reacted with an amine or amines to form

a mixture of sulfonate and sulfinate compounds.

The compounds of my invention may be used in developing solutions, especially concentrated developing solutions, as shown in the following examples which are intended only for illustration.

*Example 1*

|                                                     |       |      |
|-----------------------------------------------------|-------|------|
| Sodium- $\beta$ -hydroxyethylaminomethane sulfonate | grams | 81.5 |
| p-Methylamino-phenol sulfate                        | do    | 5.0  |
| Potassium thiocyanate                               | do    | 1.0  |
| Potassium bromide                                   | do    | 0.5  |
| Hydroquinone                                        | do    | 1.0  |
| Water to                                            | cc    | 250  |

For use this solution is made to the required volume with water.

*Example 2*

|                                                 |       |     |
|-------------------------------------------------|-------|-----|
| Di-sodium ethylenediamino-bis-methane sulfonate | grams | 73  |
| p-Methylamino-phenol sulfate                    | do    | 5.0 |
| Potassium thiocyanate                           | do    | 1.0 |
| Potassium bromide                               | do    | 0.5 |
| Water to                                        | cc    | 250 |

*Example 3*

|                                                     |       |     |
|-----------------------------------------------------|-------|-----|
| Water                                               | cc    | 385 |
| Sodium sulfite                                      | grams | 18  |
| Acetic acid (glacial)                               | cc    | 10  |
| Sodium- $\beta$ -hydroxyethylaminomethane sulfonate | grams | 531 |
| p-Methylamino-phenol sulfate                        | do    | 25  |
| Hydroquinone                                        | do    | 6   |
| Potassium bromide                                   | do    | 10  |
| Sodium thiocyanate                                  | do    | 6   |
| Glycerin                                            | cc    | 200 |
| Water to                                            | liter | 1   |

*Example 4*

|                                                     |       |     |
|-----------------------------------------------------|-------|-----|
| Sodium- $\beta$ -hydroxyethylaminomethane sulfinate | grams | 322 |
| Hydroquinone                                        | do    | 90  |
| Potassium bromide                                   | do    | 6.3 |
| Water to                                            | liter | 1   |

In a similar manner a mixture of aminomethane sulfonate and sulfinate are incorporated into a developer formula in the amount required to make concentrated developers or dry mixtures of chemicals for dissolving in water.

*Example 5*

|                                                    |       |     |
|----------------------------------------------------|-------|-----|
| Di-( $\beta$ -hydroxyethyl) aminomethane sulfonate | grams | 110 |
| p-Methylamino-phenol sulfate                       | do    | 5   |
| Potassium thiocyanate                              | do    | 1   |
| Potassium bromide                                  | do    | 0.5 |

To any of these mixtures described above may be added sodium sulfite, other developing agents, fog inhibitors, and the like.

As shown in Example 3 above, one may use sodium sulfite in conjunction with the compounds of the invention. In similar developing formulas as, for instance, those of Examples 1, 2, and 4, and in cases where mixtures of the sulfonate and sulfonate compounds are used, sodium sulfite may also be used in the required amount. I find it is advisable, especially from the standpoint of economy, to use as much sodium sulfite in the concentrated developing solutions, as is possible, and adding the compounds of the invention as solubilizers and to aid in the preservation of the solutions.

One advantageous feature of the compounds when used in developing solutions, resides in their

solubility characteristics. The compounds, especially the hydroxy alkyl derivatives, are considerably more soluble than sodium sulfite and accordingly are especially suitable for use in concentrated developing solutions. The anti-sludge properties of a developer containing compounds of my invention were demonstrated as follows: several rolls of amateur film were developed in a developing solution of the following composition:

|                              |       |     |
|------------------------------|-------|-----|
| Water, about 125° F          | cc    | 750 |
| p-Methylamino-phenol sulfate | grams | 5   |
| Sodium sulfite, dry          | do    | 100 |
| Sodium metaborate            | do    | 2   |
| Sodium thiocyanate           | do    | 1   |
| Potassium bromide            | do    | 0.5 |
| Water to                     | liter | 1   |

The same number of rolls of the same film were developed under the same conditions in a second developing solution of composition shown in Example 1 with the result that whereas a continuously heavier sludge formed in the first developer after development of a certain number of rolls of film, the second developer was nearly as clear as at first after developing the same amount of film.

As shown in Example 3, the pH of the developing solutions may be regulated by the addition of acid compounds such as meta-bisulfites, bisulfites, acid sodium acetate, acetic acid, etc., or basic compound such as sodium metaborate and the like. Suitable solid acids and bases may also be added to the dry mixtures of chemicals of my invention. Of course, the compounds of my invention also aid in the regulation of pH.

Other aminomethanesulfonates useful in developing solutions according to my invention may be prepared from aldehydes such as crotonic aldehyde, acrolein, etc., and ketones such as acetone, acetylacetone, etc., by reaction with bisulfites and amines employing suitable conditions of time and temperature.

It is to be understood that the disclosure herein is by way of example and that I consider as included in my invention all modifications and equivalents falling within the scope of the appended claims.

What I claim is:

1. A photographic developing solution comprising a developing agent and a compound selected from the group consisting of alkali salts of aminomethane sulfonates and aminomethane sulfonates.
2. A photographic developing solution comprising a developing agent and an alkali metal salt of an aminomethane sulfonate.
3. A photographic developing solution comprising a developing agent, an alkali metal salt of an aminomethane sulfonate and sodium sulfite.
4. A photographic developing solution comprising a developing agent and  $\beta$ -hydroxyethylaminomethane sulfonate.
5. A photographic developing solution comprising a developing agent and a sodium salt of ethylenediamino-bis-methane sulfonate.
6. A photographic developing solution comprising a developing agent and an alkali metal salt of an aminomethane sulfonate.
7. A photographic developing solution comprising a developing agent and an alkali metal salt of an aminomethane sulfonate and sodium sulfite.
8. A photographic developing solution comprising a developing agent and an alkali metal salt of  $\beta$ -hydroxyethylaminomethane sulfonate.

9. A solid mixture of chemicals suitable for forming a photographic developing solution by dissolving in water comprising a developing agent and a compound selected from the group consisting of alkali metal salts of aminomethane sulfonates and aminomethane sulfonates.

10. A solid mixture of chemicals suitable for forming a photographic developing solution by dissolving in water comprising a developing agent and an alkali metal salt of an aminomethane sulfonate.

11. A solid mixture of chemicals suitable for forming a photographic developing solution by dissolving in water comprising a developing agent and an alkali metal salt of an aminomethane sulfonate.

12. A solid mixture of chemicals suitable for forming a photographic developing solution by dissolving in water comprising a developing agent

and an alkali metal salt of  $\beta$ -hydroxyethylamino-methane sulfonate.

13. A photographic developing solution comprising a developing agent, an alkali metal salt of an aminomethane sulfonate, and an alkali metal salt of an aminomethane sulfonate.

14. A photographic developing solution comprising a developing agent, an alkali metal salt of an aminomethane sulfonate, and an alkali metal salt of an aminomethane sulfonate, and sodium sulfite.

15. A solid mixture of chemicals suitable for forming a photographic developing solution by dissolving in water comprising a developing agent and an alkali metal salt of an aminomethane sulfonate and an alkali metal salt of an aminomethane sulfonate.

FREDERIC R. BEAN.